

Patented Aug. 17, 1926.

1,596,020

# UNITED STATES PATENT OFFICE.

ALADAR PACZ, OF CLEVELAND, OHIO, ASSIGNOR TO THE ALUMINUM COMPANY OF AMERICA, OF PITTSBURGH, PENNSYLVANIA. A CORPORATION OF PENNSYLVANIA.

## ALUMINUM ALLOY.

No Drawing. Original application filed September 15, 1922, Serial No. 588,491. Divided and this application filed April 19, 1924. Serial No. 707,569.

This invention relates to aluminum alloys, particularly those containing silicon. Its chief object is to provide a method of making castings of such alloys which will improve their physical properties. The invention is based on the discovery that aluminum alloys, especially those containing silicon in substantial amounts, have their physical properties, especially tensile strength and ductility, improved by treatment with a reducible oxygen-containing compound of an alkali metal.

In my prior U. S. Patent No. 1,387,900, a process is described for treating aluminum-silicon alloys with fluorine compounds of an alkali metal; by that treatment the grain size of the resulting casting is greatly refined and the strength and ductility increased. It has also become known (U. S. Patent No. 1,410,461) that a similar grain-refining effect, with its consequent improvement in the physical properties of the alloys, can be effected by the introduction into the molten alloy of either metallic sodium or potassium or both. There is reason to believe that when an aluminum alloy in the molten condition is treated with an alkali fluoride, such as sodium or potassium fluoride, that a reaction takes place between the alkali metal compound and the aluminum of the alloy, which results in decomposition of the fluoride and the formation of metallic sodium or potassium in contact with the alloy. Apparently it is this alkali metal which effects the observed improvement in physical properties.

Not all alkali metal compounds are reduced by aluminum or reduced with sufficient rapidity or completeness at suitable temperatures to effect the desired changes. In addition to the class of refining compounds just referred to, and which contain fluorine, I have discovered that sodium hydroxide or potassium hydroxide, or a reducible mixture of oxygen-containing compounds of sodium or potassium will produce the desired refining effect on aluminum-silicon alloys, and under certain conditions are particularly well adapted for this purpose.

In carrying out this invention in the preferred manner, an alloy of aluminum and silicon, containing from 3 to 15 percent silicon approximately, is prepared in a suitable manner, as for example, by stirring metallic

silicon into molten aluminum and allowing it to dissolve. Aluminum base alloys containing from 8 to 13 percent silicon have especially desirable properties conferred on them by treating by my process. To the molten alloy I add sodium or potassium hydroxide equivalent to at least 0.5 percent but preferably somewhat more of free alkali metal. This compound is incorporated in the alloy, as for example, by vigorous stirring. After the reaction has been completed, the alloy is skimmed and cast in the usual manner. On standing the reduction products tend to be eliminated from the molten alloy so that eventually the capacity for improvement on casting diminishes. If the highest physical properties are desired, the molten alloy should be cast with reasonable promptness after treatment with the alkali metal oxide compound has been completed.

The sodium hydroxide can be advantageously mixed with other substances which overcome, in some degree at least, its hydroscopic tendency. For example, I may melt the caustic soda with sodium chloride, calcium fluoride, sodium fluoride, calcium oxide, etc. One convenient method of adding the sodium hydroxide or refining mixture to the alloy is to maintain a separate pot of the fused compound. A cold carbon rod or other suitable stirring rod can then be dipped into the molten sodium hydroxide, for example, and a quantity of the sodium hydroxide allowed to freeze upon the stirring rod, after which it can be transferred to the molten aluminum alloy and incorporated by vigorously stirring it therein.

Apparently the action of the aluminum is to combine with the oxygen of the sodium hydroxide to form oxide of aluminum and liberate nascent metallic sodium in contact with the alloy. It is not necessary, in fact, that sodium hydroxide be used, for other mixtures such as sodium carbonate and lime, or sodium carbonate and a reducing agent which would form the equivalent of sodium oxide in the alloy, can be effectively employed. The addition of the alkali metal in the form of a compound, rather than in elemental form, seems to be advantageous in securing thorough dissemination of the alkali metal throughout the alloy. Furthermore, the energy of the reaction seems to

serve in spreading the active principles throughout the alloy, and the reduction products other than alkali metal appear to assist in the refining action which is observed. I do not commit myself, however, in any way to any particular theory or explanation of the observed phenomenon. Neither do I limit myself to the exclusion of metals other than aluminum and silicon 10 (with their customary impurities, but include within the scope of my process such other metallic additions as may be found desirable for special purposes. Thus I have found my improved grain-refining process 15 highly advantageous in connection with the aluminum-silicon-copper alloy described and claimed in my application filed September 12th, 1919, Serial Number 323,350, and in combination with the aluminum-sili- 20 con-manganese alloy described and claimed in my application filed February 27th, 1922, Serial Number 539,740, and in combination with the aluminum-silicon-cobalt alloy de- 25 scribed and claimed in my application filed April 3rd, 1922, Serial Number 549,203.

The term alkali metal or compound as employed in the specifications and claims includes sodium and potassium only.

The invention herein set forth has been 30 disclosed in my pending application Serial No. 588,491 filed September 15, 1922, of which this is a division.

Having thus described my invention so that those skilled in the art may practice 35 the same, what I desire to secure by Letters Patent is defined in what I claim.

What I claim is:

1. The method of making aluminum base 40 alloy castings comprising preparing an alloy containing not less than about 3 percent nor more than 15 percent of silicon, treating the molten alloy with a reagent containing an oxygen-containing compound of an alkali metal capable of being reduced 45 in the molten alloy, and causing the alloy to solidify while it still contains sufficient of the reduction products to produce an improvement in the physical properties of the alloy.

2. The method of making aluminum base 50 alloy castings comprising preparing an alloy containing from about 8 to 13 percent of silicon, treating the molten alloy with a re- 55 agent containing an oxygen-containing com- pound of an alkali metal reducible in the molten alloy, and casting the alloy while it still retains sufficient of the reduction prod- ucts to favorably affect the physical proper- ties of the alloy.

3. The method of making aluminum base 60 alloy castings comprising preparing an alloy

containing not less than about 3 percent nor more than about 15 percent of silicon, treating the molten alloy with a reagent containing sodium hydroxide, and causing the alloy to solidify while it still contains sufficient of the reduction products to produce an improvement in the physical properties of the alloy.

4. The method of producing aluminum 70 base alloys which contain silicon in substantial amount, which comprises the step of introducing into the molten alloy a reagent including a reducible oxygen containing compound of sodium capable of being reduced in the molten alloy.

5. The method of producing aluminum base alloys containing silicon in substantial amount, which comprises the step of introducing into the molten alloy a reagent comprising alkali metal hydroxide.

6. The method of producing aluminum base alloys containing silicon in substantial amount, which comprises the step of introducing into the molten alloy a reagent comprising sodium hydroxide.

7. The method of making aluminum silicon alloy castings having improved physical properties which comprises preparing a molten alloy containing a substantial amount 90 of silicon, incorporating in the molten alloy an oxygen-containing compound of an alkali metal capable of being reduced in the molten alloy, and then casting the alloy with reasonable promptness.

8. The method of making a silicon-containing aluminum alloy casting having improved physical properties which comprises preparing a molten alloy containing a substantial amount of silicon, melting a reagent containing a reducible, oxygen-containing compound of an alkali metal, coating a stirring rod with the molten reagent, transferring the coated rod to the molten alloy and stirring the molten metal therewith, and casting the alloy with reasonable promptness after the stirring.

9. The method of making a silicon-containing aluminum alloy casting having improved physical properties which comprises preparing a molten alloy containing a substantial amount of silicon, treating the molten alloy with an oxygen-containing alkali metal compound capable of being reduced to metallic form in the molten alloy, and casting the alloy before substantially all the reduction products have been eliminated therefrom.

In testimony whereof I hereunto affix my signature this 16th day of April, 1924.

ALADAR PACZ.